

## UNITED STATES PATENT OFFICE

2,318,096

## TRANSFER SHEET

Frederick A. Quick, Bellerose, N. Y., assignor to  
All Purpose Gold Corporation, Brooklyn, N. Y.,  
a corporation of New York

No Drawing. Application September 4, 1940,  
Serial No. 355,375

7 Claims. (Cl. 117—36)

This invention relates generally to transfer sheets, that is to sheets from which material may be transferred to a receiving surface by suitable treatment. More particularly this invention relates to transfer sheets the transferable matter on which is in the form of an unbroken film of solid material, desired portions of which may be transferred to a receiving surface by the application of pressure and without any other treatment or the application of heat or solvents.

Coordinate therewith my invention relates to a method of making a transfer sheet of the character mentioned.

Before discussing my invention in detail I will premise that my improved transfer sheet comprises a sheet, hereinafter called the "carrier sheet" on which is imposed a coating, hereinafter referred to as the "transferrable film," portions of which may be caused to adhere to a surface, hereinafter referred to as the "receiving surface" by applying pressure to the reverse side of the carrier sheet so as to press it against the receiving surface.

In its illustrative embodiment and practice selected for disclosure in this application my invention has been described in its application to so-called "album paper," which is a rough-surfaced, black paper ordinarily used in photograph albums for mounting photo prints thereon and also used in the moving picture film industry for the writing of titles thereon. While it has been so described, it will be understood that my invention is not necessarily so restricted, but may have application to other kinds of paper and to surfaces of material other than paper. Nor is it necessarily restricted to material that is black in color.

When it is desired to inscribe matter such as a title or to apply decorative matter on such album paper, it is customary, according to the present conventional practice, to use white ink (Chinese white) or white crayon.

Both of these media leave much to be desired. With white ink uniformity is difficult of attainment, and then only with the greatest care, and unless such uniformity is attained it is difficult to obtain satisfactory photographic reproduction, which of course is essential where the ink is used on a moving picture film. To these disadvantages must be added the inconvenience of keeping on hand equipment comprising liquid ink and the necessary assortment of brushes and pens.

White crayon on the other hand leaves a greasy surface and the markings are not uniform and

have a grayish appearance for which reason they are unsuitable for photographic reproduction.

These disadvantages are overcome by my invention which has all the convenience of use of carbon paper and which gives clear and distinct markings of uniform appearance and which are constituted by portions of a solid film. In the particular application of my invention herein disclosed the markings are continuous, opaque, white film portions, which stand out sharply and distinctly from the black back-ground.

It is the general object of my invention to provide in a transfer sheet of the character described, a simple, effective and inexpensive composition and structure and further to provide a simple effective and inexpensive method for manufacturing such a sheet.

It is among the more particular objects of my invention to provide in a transfer sheet of the character described a carrier sheet and a transferable film on said carrier sheet having such adhesive properties that whenever pressure is applied to the reverse side of the carrier sheet so as to press the film side against a receiving surface, a portion of said transferable film will separate from the carrier sheet and will adhere to the receiving surface, and the portion of the film so transferred will be substantially coextensive with the area to which the pressure has been applied. It is further among the more particular objects of my invention to provide in a transfer sheet a transferable film having opposed surfaces the adhesive properties of which are not the same.

It is also among the more particular objects of my invention to provide in a transfer sheet a transferable film the adhesion of which to the carrier sheet is less than its adhesion to a receiving surface, and further a transferable film the cohesive properties of which are such in relation to its adhesive properties, that pressure of portions thereof against a receiving surface will cause only those portions to separate from the carrier and from the other parts of the film and to adhere to the receiving surface, while those portions to which no pressure has been applied will remain in adhesive contact with the carrier film.

These objects and such other objects as will hereinafter appear or be pointed out are attained in the illustrative embodiment and practice of my invention now to be disclosed.

My improved transfer sheet may be most conveniently described in connection with the process of its manufacture.

As a base or carrier sheet I use a sheet of ma-

terial that has surface characteristics so related to the transferable film to be imposed thereon that it will permit separation of the film from the carrier sheet under the conditions of use, and said material having sufficient flexibility, toughness, hardness and cohesion so that it will not break or tear when the stylus or other pressure instrument is applied thereto, but will yield sufficiently to transmit the pressure from its reverse surface, to which the pressure is applied, to the transferable film.

The thickness of the sheet is another important factor to be considered. If the sheet is too thin it will tear readily; if too thick it cannot be used to transmit localized pressure, such as is required in transferring portions of film having a desired configuration.

I have found "Cellophane" to be a material satisfactory in actual practice. Where "Cellophane" is used for the carrier sheet the best results were obtained with a thickness of four and one-half one-thousandths of an inch.

Oiled silk and certain kinds of paper may also be mentioned among materials suitable for my purpose. Cellulose acetate is also suitable but is not adapted for a continuous process of manufacture in which the material is used in rolls, as it becomes soft under the action of the solvents used in applying the coating. However, it can be used in sheet form and the coating can be applied by brush.

To one side of this carrier sheet is applied the transferable film, which, as already mentioned, is to possess the property of adhering to a receiving surface and separating from the carrier sheet under pressure applied to the reverse side of the latter, and further as having such cohesive properties that only the portions pressed on will so adhere and separate. The pressure that is to effect separation may be either a gliding pressure as by applying a stylus, or an impact pressure, as by the keys of a typewriter.

As the base for such a coating I have found shellac gum to be suitable. This is modified by the addition of other gums to obtain the desired adhesive and cohesive properties, and further has suitable plasticizers added thereto to obtain and maintain the desired consistency. In order to give body to the coating and to obtain opacity, or color where that is desired, pigments are also added.

For purposes of application an alcoholic solution of these ingredients is conveniently made.

In order to obtain adhesive characteristics that are different for the two surfaces of this film I make it in two layers or coats, the first of which may be a main layer, that gives body to the film and determines its cohesive properties, while the second is a coating for one surface of this main layer that is intended to change the adhesive properties of that surface.

When application of this film is made by an alcoholic solution, alcohol soluble gums are required. It will be understood, however, that my invention also contemplates solution in other solvents and the use of gums soluble therein even though not soluble in alcohol, provided they are suitable for the attainment of the objects of my invention.

I have found that when shellac gum and sandarac gum are used in the first coat together with pigments the qualities requisite in the second coat are attained by the use of shellac gum and Pontianak gum.

As a preferred formula for the first coat I may give the following:

|               |        |    |
|---------------|--------|----|
| Shellac gum   | oz.    | 12 |
| Sandarac gum  | oz.    | 8  |
| Ethyl alcohol | quarts | 10 |
| Butyl alcohol | do     | 1  |
| Glycerine     | oz.    | 4  |
| Castor oil    | oz.    | 2  |

10 Into these ingredients, after mixing is ground a pigment comprising:

|                  | Pounds |
|------------------|--------|
| Titanium dioxide | 2      |
| Zinc oxide       | 1      |
| 15 Chalk         | 1/2    |
| China clay       | 1/2    |

This grinding operation, when performed in a mill, is complete in about one hour.

The quantities given have been found sufficient to cover about 800 square feet of the carrier sheet.

The coated sheet is then dried at a temperature of about 120° Fahrenheit and the drying process when performed by passing the sheet through a drying tunnel, has been found to take about two and one half minutes.

A preferred formula for the second coat is the following:

|                   |        |    |
|-------------------|--------|----|
| Shellac gum       | oz.    | 6  |
| Pontianak gum     | oz.    | 2  |
| Ethyl alcohol     | quarts | 10 |
| Toluol            | oz.    | 10 |
| Ethyl acetate     | oz.    | 10 |
| Methyl alcohol    | oz.    | 10 |
| Glycerine         | oz.    | 16 |
| Dibutyl phthalate | oz.    | 13 |

This quantity has been found sufficient to coat about 2,000 square feet.

10 This coat is dried at a temperature of about 150° Fahrenheit. When carried in a drying tunnel this operation has been found to take about two and one-half minutes.

Thereafter the rolls or sheets may be cut into sizes suitable for sale and may be otherwise treated to prepare it for the market.

It will be understood that the quantities given in the above formulas may be departed from and still give satisfactory results, although the best 50 results are obtained when the exact quantities are used. I have obtained satisfactory results when the quantities given are varied 10%.

As an added feature of my invention I may coat the reverse (or uncoated) side of the carrier 55 sheet with a waterproof coating. With such a coating I find that the lasting qualities of my improved transfer sheet are greatly improved.

Where the reverse side is to be written on I have found that a better writing surface is secured by applying a coating of nitrocellulose lacquer to this reverse side.

If desired the coating on the reverse side may combine the two qualities of being waterproof and providing a better writing surface.

65 In using my improved transfer sheet it will be understood that it is laid face down on the receiving surface, that is so that the transferable film lies in contact with the receiving surface and some suitable instrument such as a stylus or a pencil traces the matter that is to appear 70 on the receiving surface on the reverse side of the carrier sheet, the tracing operation being accompanied by pressure of the instrument on the carrier sheet. Thereby a separation of the portions of the transferable film underlying the por-

tions of the carrier sheet to which pressure has been applied from the carrier sheet, and its adhesion to the receiving surface, are effected.

Where the carrier sheet is transparent the course of the tracing operation will be readily observable during the operation due to the changed appearance of the sheet as the opaque transferable film portions become separated from the transparent carrier sheet.

Where this effect is not desired it is obviously not necessary to use a transparent carrier sheet, such as transparent "Cellophane," and opaque or semi-opaque or translucent materials or materials having opaque or semi-opaque or translucent coats thereon may be used in the carrier sheet.

Obviously instead of the tracing operation being performed directly on the reverse side of the carrier sheet a pattern sheet may be superposed thereover and the tracing operation performed the tracing and pressure operation carried out by following the pattern on the pattern sheet.

From what has already been said it will also be obvious that instead of a white transferable film my improved transfer sheet lends itself to production in any desired color and that it is not necessarily restricted to opaque films, but that for particular purposes transparent or translucent transferable films may be found preferable.

While I have herein disclosed one illustrative embodiment of my invention and one illustrative manner of practising the same, it will be understood that it may be embodied in many forms and practised in many other ways, as will be obvious to those skilled in the art, and that the disclosure herein is by way of illustration merely and is not to be interpreted in a limiting sense, and that I do not limit myself other than as called for by the appended claims.

Having thus described my invention and illustrated its use, what I claim as new and desire to secure by Letters Patent, is:

1. A transfer sheet comprising a carrier sheet of "Cellophane" and a transferable film on one side thereof, said film comprising two layers, the first being produced by the application of an alcoholic varnish composed of

|               |     |    |
|---------------|-----|----|
| Shellac gum   | oz  | 12 |
| Sandarac gum  | oz  | 8  |
| Ethyl alcohol | qts | 10 |
| Butyl alcohol | qt  | 1  |
| Glycerine     | oz  | 4  |
| Castor oil    | oz  | 2  |

in which is suspended

|                  |     |     |
|------------------|-----|-----|
| Titanium dioxide | lbs | 2   |
| Zinc oxide       | lb  | 1   |
| Chalk            | lb  | 1/2 |
| China clay       | lb  | 1/2 |

applied at the rate of about 800 square feet of surface for the quantity given, and the second coat being produced by the application of an alcoholic varnish composed of

|                   |     |    |
|-------------------|-----|----|
| Shellac gum       | oz  | 6  |
| Pontianak gum     | oz  | 2  |
| Ethyl alcohol     | qts | 10 |
| Toluol            | oz  | 10 |
| Ethyl acetate     | oz  | 10 |
| Methyl alcohol    | oz  | 10 |
| Glycerine         | oz  | 10 |
| Dibutyl phthalate | oz  | 16 |

at the rate of about 2,000 square feet for the quantity given.

2. A transfer sheet comprising a carrier sheet of "Cellophane" having a waterproof coating on one side and a transferable film on the other side thereof, said film comprising two layers, the first being produced by the application of an alcoholic varnish composed of

|               |     |    |
|---------------|-----|----|
| Shellac gum   | oz  | 12 |
| Sandarac gum  | oz  | 8  |
| Ethyl alcohol | qts | 10 |
| Butyl alcohol | qt  | 1  |
| Glycerine     | oz  | 4  |
| Castor oil    | oz  | 2  |

in which is suspended

|                  |     |     |
|------------------|-----|-----|
| Titanium dioxide | lbs | 2   |
| Zinc oxide       | lb  | 1   |
| Chalk            | lb  | 1/2 |
| China clay       | lb  | 1/2 |

applied at the rate of about 800 square feet of surface for the quantity given, and the second coat being produced by the application of an alcoholic varnish composed of

|                   |     |    |
|-------------------|-----|----|
| Shellac gum       | oz  | 6  |
| Pontianak gum     | oz  | 2  |
| Ethyl alcohol     | qts | 10 |
| Toluol            | oz  | 10 |
| Ethyl acetate     | oz  | 10 |
| Methyl alcohol    | oz  | 10 |
| Glycerine         | oz  | 16 |
| Dibutyl phthalate | oz  | 13 |

at the rate of about 2,000 square feet for the quantity given.

3. A transfer sheet comprising a carrier sheet and a transferable film on one side thereof, said film comprising two layers, the first being produced by the application of an alcoholic varnish composed of

|               |     |    |
|---------------|-----|----|
| Shellac gum   | oz  | 12 |
| Sandarac gum  | oz  | 8  |
| Ethyl alcohol | qts | 10 |
| Butyl alcohol | qt  | 1  |
| Glycerine     | oz  | 4  |
| Castor oil    | oz  | 2  |

in which is suspended

|                  |     |     |
|------------------|-----|-----|
| Titanium dioxide | lbs | 2   |
| Zinc oxide       | lb  | 1   |
| Chalk            | lb  | 1/2 |
| China clay       | lb  | 1/2 |

applied at the rate of about 800 square feet of surface for the quantity given, and the second coat being produced by the application of an alcoholic varnish composed of

|                   |     |    |
|-------------------|-----|----|
| Shellac gum       | oz  | 6  |
| Pontianak gum     | oz  | 2  |
| Ethyl alcohol     | qts | 10 |
| Toluol            | oz  | 10 |
| Ethyl acetate     | oz  | 10 |
| Methyl alcohol    | oz  | 10 |
| Glycerine         | oz  | 16 |
| Dibutyl phthalate | oz  | 13 |

at the rate of about 2000 square feet for the quantity given.

4. The method of manufacturing a transfer sheet which comprises the steps of applying to

one side of a thin sheet of smooth, transparent Cellophane a solution comprising

|               |     |    |
|---------------|-----|----|
| Shellac gum   | oz  | 12 |
| Sandarac gum  | oz  | 8  |
| Ethyl alcohol | qts | 10 |
| Butyl alcohol | qt  | 1  |
| Glycerine     | oz  | 4  |
| Castor oil    | oz  | 2  |

in which is suspended a pigment comprising

|                  |      |     |
|------------------|------|-----|
| Titanium dioxide | lbs. | 2   |
| Zinc oxide       | lb.  | 1   |
| Chalk            | lb.  | 1/2 |
| China clay       | lb.  | 1/2 |

at the rate of about 800 square feet of surface for the quantity given and drying said coating at a temperature of the order of 120° Fahrenheit, then applying over the coating so produced a solution comprising

|                   |     |    |
|-------------------|-----|----|
| Shellac gum       | oz  | 6  |
| Pontianak gum     | oz  | 2  |
| Ethyl alcohol     | qts | 10 |
| Toluol            | oz  | 10 |
| Ethyl acetate     | oz  | 10 |
| Methyl alcohol    | oz  | 10 |
| Glycerine         | oz  | 16 |
| Dibutyl phthalate | oz  | 13 |

at the rate of about 2000 square feet of surface for the quantity given, and drying said sheet at a temperature of the order of 150° Fahrenheit.

5. The method of manufacturing a transfer sheet which comprises the steps of applying to a carrier sheet a first coat comprising shellac gum and sandarac gum in solution together with plasticizers and pigments, drying said coat and superposing on said first coat a coat comprising shellac gum and Pontianak gum in solution together with plasticizers and drying said coating.

6. The method of manufacturing a transfer sheet which comprises the steps of applying to a carrier sheet a solution comprising shellac gum and sandarac gum and then applying a second solution comprising shellac gum and Pontianak gum.

7. The continuous process of manufacturing a transfer sheet which comprises applying to a roll of material constituting a carrier sheet, by means of a roller coater, a first coat comprising shellac gum, sandarac gum and pigments, drying said coat by passing it through a drying tunnel, applying a second coat comprising shellac gum and Pontianak gum by means of a roller coater, and drying said second coat by passing it through a drying tunnel.

FREDERICK A. QUICK.